

# UNITED STATES PATENT OFFICE.

HAROLD R. EYRICH, OF PHOENIXVILLE, PENNSYLVANIA, AND JOHN A. SCHREIBER, OF CHICAGO, ILLINOIS, ASSIGNORS TO THE PAPER DE-INKING CO., OF CHICAGO, ILLINOIS, A CORPORATION OF ILLINOIS.

## METHOD FOR REMOVING INK FROM PRINTED PAPER.

1,421,195.

Specification of Letters Patent. Patented June 27, 1922.

No Drawing.

Application filed April 27, 1921. Serial No. 465,026.

To all whom it may concern:

Be it known that we, HAROLD R. EYRICH, and JOHN A. SCHREIBER, citizens of the United States, HAROLD R. EYRICH residing 5 at Phoenixville, Pennsylvania, and JOHN A. SCHREIBER, residing at Chicago, Cook County, Illinois, have invented a certain new and useful Improvement in Methods for Removing Ink from Printed Paper, of 10 which the following is a specification.

This invention relates to the art of de-inking print-paper and has for its object 15 to provide a method whereby the ink may be expeditiously and economically removed from the paper, to the end that such paper may be used as paper stock to produce a clean white print-paper of good quality or given any suitable or desired color.

It has heretofore been proposed to deink 20 paper by treating printed paper pulp with bleaching agencies in connection with colloidal substances, such as silicic acid, silicates and alumina compounds. It has also been proposed to subject the paper to the 25 action of chemicals which produce a soap, such as soda, margaric acid, and oleic acid, together with an absorbent earthy matter. Another method has been to subject the macerated or pulped paper stock containing 30 the ink to the action of an alkali in solution, together with a silicate of aluminum such as fuller's earth, kaolin or other clays, silicate of magnesium such as talc, soap-stone, etc., and then washing the fiber.

All of these methods have proved unsatisfactory or inefficient in the practical art, not only because they did not thoroughly 35 remove the ink but because the amount of materials necessarily employed and the extent of time required by the process rendered the cost so high that there was no economy in recovering the old stock as against the use of new stock. By the process hereinafter described, we are enabled 40 to expeditiously and thoroughly remove the ink from the printed paper stock and produce a thoroughly satisfactory white print-paper therefrom, superior to any paper heretofore made from print-paper stock and 45 at a cost materially below that of paper made from new stock, and thus effect a saving not only in the price of the paper reproduced therefrom but also effect economy in the consumption of the raw materials that 50

would be required if all new paper stock 55 was employed.

We have discovered that, if printed paper pulp is treated with an alkali to decompose or break up the ink and then is subjected to a colloidal solution of the substance 60 known as bentonite (of which there are a number of varieties), and then thoroughly washed, preferably in running water, the ink is thoroughly and expeditiously removed and the pulp left in a most excellent condition 65 for the manufacture of a good grade of print-paper.

The inventive idea involved is capable of some variations and modifications without departing from the essential spirit of the 70 invention and, for the purpose of illustrating the invention, we herein describe one specific and the best form now known to us, but we wish it distinctly understood that the specific process set forth is for the purpose 75 of clearly describing the invention and is not designed to define the limits of the invention, reference being had to the claims for this purpose.

The process may be performed with any 80 suitable apparatus, but preferably a quantity of shredded printed paper is placed in a "beater", together with an alkali material such as sodium hydroxide, sodium carbonate, ammonia, borax, or the like, to break 85 up the binder material of the printer's ink, and a quantity of bentonite, with an adequate supply of water. Bentonite in water forms a substantially permanent colloidal solution, and the alkaline material employed 90 of course passes into solution in the water so that there is formed what we term an alkaline solution of bentonite. The alkali acts to decompose or break up the ink by reason of its action upon the grease or oily content 95 of the ink, thus freeing the pigment of the ink which is taken up by the bentonite. After the pulp has been thoroughly agitated and stirred in the "beater", to the end that these actions may take place, the pulp is 100 then thoroughly washed, preferably in running water, which carries away the alkaline bentonite solution and with it the constituents of the ink. This washing is continued until the ink is thoroughly removed. In 105 order to neutralize any alkaline condition that may remain in the paper pulp after the washing, it is then treated with any suitable

alkali neutralizer, as an acid, such as sulphuric acid ( $H_2SO_4$ ), or an acid salt. This also acts to brighten the color. If desired, sizing material is then added and, if the paper is to be colored, a suitable dye, as well as alum, and when thoroughly mixed the pulp is then remade into paper in any suitable or usual manner.

One specific formula which we have found to be highly efficient and satisfactory consists in using approximately 300 pounds of bentonite, 200 pounds of sodium carbonate, and 8,000 gallons of water to the ton of old newspaper to be treated. Another specific formula which we have also found advantageous consists in using approximately 150 pounds of bentonite, 32 pounds of sodium carbonate, 20 pounds of lime, and 8,000 gallons of water to the ton of old newspaper to be treated. The process may be carried out at ordinary temperatures, but the desired result is more expeditiously effected if the temperature of the initial charge is raised to a degree not to exceed 120° F. and then applying the cold washing water.

While there are several varieties of bentonite which may be employed, we have found the variety known as "wilkinite" to be highly efficacious.

Bentonite is to be distinguished from clays such, for example, as fuller's earth and kaolin, in that with neither of these can a permanent colloidal solution be obtained, since the particles of the clay rapidly settle out from the solvent such as water, whereas bentonite forms a substantially permanent colloidal solution, probably due not only to the fact that it is a different substance but also to its different physical characteristics, the particles of bentonite being extremely small, 70% (according to H. W. Wiley) being less than .0015 millimeters in diameter.

Whatever the reasons may be, we have discovered that an alkaline solution of bentonite effectively and rapidly deinks the paper stock so as to render the process commercially practicable, whereas, so far as we are informed, all of the prior methods pro-

posed with this object in view have been abandoned in commercial practice, either because of their inefficient action in deinking, or the time and cost of the practice, or both.

What is claimed is:—

1. The process of deinking paper which consists in subjecting the paper to an alkaline solution of bentonite.

2. The process of deinking paper which consists in decomposing the ink, treating the mass in a bentonite solution and then washing the mass.

3. The process of deinking paper which consists in subjecting the paper pulp to the action of an alkaline solution of bentonite and then washing the pulp.

4. The process of deinking paper which consists in mixing the paper, an alkali, and bentonite, agitating the mixture in the presence of water, and then draining off the water.

5. The process of deinking paper which consists in subjecting paper pulp to the action of an alkali and a bentonite solution in the presence of water, draining off the water and then washing the pulp.

6. The method of deinking paper which consists in subjecting the paper to the action of an alkali and then treating it with a bentonite solution.

7. The method of deinking paper which consists in decomposing the ink and then treating the mass with a bentonite solution.

8. The process of deinking paper which consists in subjecting paper pulp to the action of an alkaline solution of bentonite, then washing the pulp, and then adding an acidulous material to neutralize any remaining alkalinity.

9. The process which consists in subjecting paper pulp to the action of an alkaline solution of bentonite, then washing the pulp, and then neutralizing any remaining alkalinity.

In witness whereof, we have hereunto subscribed our names.

HAROLD R. EYRICH.  
JOHN A. SCHREIBER.